

## UNITED STATES PATENT OFFICE

HENRY DREYFUS, OF LONDON, ENGLAND

## PROCESS FOR THE PRODUCTION OF CELLULOSE ESTERS

No Drawing. Application filed November 30, 1925, Serial No. 72,403, and in Great Britain October 30, 1925.

This invention relates to the production of cellulose acetate or other cellulose esters.

In my French specification No. 565,654, and my U. S. application Serial No. 633,016, I have described inter alia how cellulosic materials may be pretreated with organic acids, such as acetic acid or formic acid and the like, at ordinary or raised temperatures or with cooling before subjecting them to acetylation or other esterification, while in U. S. application Serial No. 747,054 and British application No. 22697/24 I have described how such pretreatment with organic acids may be preceded, particularly in the case of cellulosic materials other than cotton such as wood pulps, by a treatment with alkaline substances to render the materials more reactive to acetylation or other esterification.

Further in U. S. application Serial No. 66,103 and British application No. 24,867/25 I have described how the pretreatment may be carried out with vapors of the organic acids, particularly lower fatty acids such as formic or acetic acid, the vapors being employed alone or in admixture with air or other inert gas, or being generated by soaking the materials in the concentrated or dilute acids and subsequently passing air or other inert gas through the materials. Preferably after the treatment air or other inert gas is passed through the materials to remove the organic acid wholly or partially.

Hitherto it has not been possible to obtain useful cellulose esters or cellulose acetate by esterifying or acetylating cellulose in absence or substantially in absence of benzol or other liquid diluents (i. e. by esterifying or acetylating cellulose in the solid or natural fibrous state in absence or substantially in absence of benzol or other liquid diluents, and in absence of liquid solvents or in presence of such small quantities of liquid solvents that the cellulose acetate or other cellulose ester is produced substantially in the solid or fibrous state and not in form of its solution). This was due to many reasons, such as, amongst others, the quantities of condensing agent (such as sulphuric acid) employed, which gave rise to so much heat

that the products obtained were of little or no practical value.

I have now found that cellulosic materials, pretreated with organic acids as described in my patents and applications referred to above, owing to their greatly increased reactivity, may be esterified or acetylated in absence or substantially in absence of benzol or other liquid diluents, to yield highly useful cellulose esters or cellulose acetate. This is an enormous advantage as it enables dispensing with most of the liquor used and further no precipitation from acetylizing or other esterifying solution is necessary. Further, the acetylation or other esterification products produced are much more homogenous and cleaner and present many other advantages which will be evident and require no mention here.

According to the present invention I produce cellulose acetates or other cellulose esters by subjecting cellulosic materials which have previously been subjected to pretreatment with organic acids in the manner indicated in my previous patents and applications referred to above, to acetylation or esterification in "suspension" in absence or substantially in absence of benzol or other liquid diluents. (That is, the cellulosic material is subjected to acetylation or esterification in their natural or fibrous state in absence or substantially in absence of benzol or other liquid diluents and in absence of liquid solvents or in presence of such small quantities of liquid solvents that the cellulose acetates or other cellulose esters are produced substantially in the solid or fibrous state and not in form of their solution). The acetylation or other esterification is effected by passing the vapours of the acetylating or other esterifying agent or agents, over or through the said cellulosic materials.

The reaction is preferably performed in presence of condensing agents, and particularly sulphuric acid, by first impregnating the cellulosic materials in any suitable manner with the condensing agent or agents. Other methods of applying the condensing agents may however be employed as hereinafter explained, or the

reaction may be carried out without condensing agents. Further the vapors of the acetylating or other esterifying agent or agents may be mixed with vapors of solvents, such as acetic acid vapor, and with air or other indifferent gas or gases.

In performing the invention, I may first impregnate the aforesaid preheated cellulosic materials with a relatively small or reduced quantity of condensing agent, such as sulphuric acid, for example about  $\frac{1}{2}\%$  to 3% on the weight of the cellulosic materials, for instance by impregnating with a solution of the condensing agent in water or acetic acid and then removing partially or entirely the acetic acid or water by pressing out, hydro-extracting, or drying, or by passing a stream of air or other indifferent gas or gases through the material, or even moisture in the form of acetic acid or some water may be left in the material.

It is of course understood that pretreatment with organic acids such as acetic acid in the liquid state may, if desired, be combined with the impregnation with the condensing agent and be performed for example in the manner indicated in my previous French Patent 565654 or my U. S. application S. 633,016, after which—and prior to acetylation or other esterification—the acetic or other organic acid is removed partially or entirely in the manner above indicated, i. e. by pressing out, hydro-extracting, by drying or by passing air or other indifferent gas or gases through the material.

Instead of employing relatively small or reduced quantities of condensing agent or agents, I may employ larger quantities, but the employment of larger quantities is not attended with any advantages.

After impregnation the cellulosic material may be submitted to acetylation or other esterification by passing over or through said material the vapours of the acetylating or other esterifying agent or agents in presence or absence of vapours of organic acids, such as acetic acid, and preferably in admixture with air or like indifferent gas or gases. Thus, for example, I may employ a mixture of air or other indifferent gas or gases and acetic anhydride vapour, or a mixture of air or other indifferent gas or gases and the vapours of acetic anhydride and acetic acid. Such mixtures may be formed in any suitable way as, for instance, by simply mixing the gases and vapour, but preferably they are formed by passing air or other indifferent gas or gases through acetic anhydride or acetic anhydride mixed with acetic acid in the cold or with heating. The cellulosic materials are preferably subjected to constant moving or agitation mechanically during the acetylation or other esterification, as for instance by subjecting them to the action of the said vapours or mixtures of said vapours and air

or the like in revolving drums or the like. Less preferably the reaction may be performed without this agitation or moving.

The reaction may if desired be performed with heating, the cellulosic materials and/or the said vapours (or mixtures containing the same) being heated; the reaction may, however, be also performed without heating, though without heat the reaction may take longer to perform.

Further, if condensing agents of a volatile nature are employed, they may be passed together with the vapours of the acetylating or other esterifying agent (or mixtures of said vapours with air or other indifferent gas or gases) over or through the cellulosic material, whether or not said cellulosic material has previously been impregnated with catalysts. Even sulphuric acid may be employed in this manner, as it is to a certain extent volatile. From a practical point of view, however, there is no advantage in employing sulphuric acid in this manner as the reaction is too slow.

If desired the vapours of the acetylating or other esterifying agent or agents may be passed over or through the cellulosic materials without being admixed with air or other indifferent gas or gases, for instance by passing said vapours (whether containing catalyst vapours or acetic acid vapours and the like or not) over or through said cellulosic materials under suction or vacuum.

The vapours, whether employed in admixture with air or other gas or gases or not, may be subjected to processes for recovery after passing over or through the cellulosic materials, or they may be circulated or passed again over the cellulosic materials until the acetylating or esterifying agent is exhausted partially or entirely; preferably after passing over or through the cellulosic materials and prior to being repassed or circulated, the vapours are adjusted to compensate changes in their constitution incurred in the reaction. Thus, for example, when acetic anhydride alone or in admixture with air or other indifferent gas or gases and mixed or not with acetic acid vapour, is passed over or through the cellulosic materials, the issuing vapours will contain a certain amount of acetic anhydride, but before passing the vapours again over or through the cellulose materials it is preferable to add more acetic anhydride to the vapours to compensate for the acetic anhydride used up in the reaction; however, the vapours may be passed without further additions until the anhydride is substantially exhausted.

The reaction may be continued until the desired degree of acetylation or esterification has been reached, which may be found for example by analysis of the products or tests as to their solubility in the desired solvent or solvents.

The above instances of methods of performing the invention are of course given only by way of illustration and are in no way limitative.

As cellulosic materials for the purpose of the present invention, I may employ cotton (mercerized or non-mercerized), wood pulps (for instance wood pulp which has been previously submitted to a treatment with alkali, or alkaline substances such as barium hydroxide, sodium zincate, sodium aluminate, or organic bases especially the alkaline treatment indicated in my previous British application No. 22697/1924 and U. S. application S. 747,054) or other cellulosic materials or conversion products which have been submitted to the hereinbefore indicated pretreatments whether or not such pretreated materials have been deprived, prior to the acetylation, substantially or entirely of acetic acid where acetic acid is used for the said pretreatments. Thus, where acetic acid is used either in vapour form or in the liquid state for the hereinbefore indicated pretreatments, the cellulosic materials may be optionally deprived (partially or entirely) of the acetic acid prior to acetylation or other esterification, for example by subjecting them to a stream of air or other indifferent gas or gases, or when liquid acetic acid is used, by hydro-extraction, pressing out or the like, with or without subsequent subjecting to a stream of air or other indifferent gas or gases. When formic acid is used for the hereinbefore indicated pretreatments the cellulosic materials are preferably deprived (for example in a manner analogous to that indicated for acetic acid above) of the formic acid prior to acetylation or other esterification, to avoid reactions with the acetic anhydride or other esterifying agent or agents. The cellulose acetates or other cellulose esters produced by the process of the present invention may, if desired, be subjected to secondary treatments or reactions for the purpose of changing their solubilities, either before or after stabilization and/or elimination or neutralization of the condensing agents. Such secondary treatments or reactions may be performed in suspension or after first dissolving the cellulose acetate or other esters in acetic acid or other solvents. Preferably, however, I perform the secondary treatment by subjecting the cellulose derivatives, after the acetylation or other esterification, to the action of vapours of formic or acetic acid (or mixtures thereof) containing sufficient humidity to destroy any anhydride or other esterifying agent remaining in the cellulose derivatives or even containing excess of humidity or water vapour. Or less advantageously I may employ water vapour or humidity alone, employing, for example, reduced quantities of water vapour in ad-

mixture with air or like indifferent gas or gases.

The vapours may be passed over or through the materials in a manner analogous to that employed in the acetylation or esterification process, i. e. they may be employed in admixture or not with air or other indifferent gas or gases and passed over or through the cellulose derivatives, preferably while subjecting the latter to moving or agitation, for example in revolving drums or the like. Further, vapours of hydrochloric acid, nitric acid vapours, or other vapours may, if desired, be employed in admixture with the organic acid vapours or water vapours. Thus for example I may employ vapours of acetic acid or formic acid (or mixtures thereof) loaded with some hydrochloric acid vapour or nitric acid or other vapour, in presence or absence of more or less humidity promoting solubility changes. Preferably I employ such mixtures in the cold and by passing them in admixture with air or other indifferent gas or gases when mineral acids vapours are used, but when employing organic acids such as acetic acid I may heat up to temperatures such as 70° to 100° C., so as to accelerate the reaction.

The above special form of execution of the secondary treatments or reaction is of course given only by way of illustration and is in no way limitative.

Further, I may perform the secondary treatments or reactions after first dissolving up the cellulose derivatives in acetic acid or other solvents, or after first forming suspensions of the cellulose derivatives, for example by adding benzol or like diluents in presence or absence of acetic acid or the like. In such cases the secondary treatments or reactions may be performed for example by the methods described in my prior British Patents Nos. 20,852/1912, 207,562, my U. S. reissue Patent 14,338 and my U. S. application S. 633,016, and my British Patent 20,977/1911 and U. S. Patent 1,217,722, the two latter of which in particular describe in detail processes of further treatment for transforming primary acetylation products into products having other solubilities as desired, and to which I refer for the sake of brevity. In these specifications above referred to I have shown how the primary esterification products or their esterification solutions or otherwise made up solutions of them, or in suspension, can be thus transformed by using the direct acetylation solutions or other solutions of the primary esterification products, with or without the addition of water or other similarly acting agents having the effect of destroying acetic anhydride and which at the same time should preferably be able to be themselves esterified without producing water in any way even intermediately, as for instance lactic acid (the absence of water or

similarly acting agents in the treatment or the quantity of water or similarly acting agents used directing the phases of solubilities passed through).

5 I have also there described how the esterification solutions can be treated by neutralizing the effect of the condensing agent partially or completely and be submitted in such form to a secondary treatment either 10 at ordinary temperature or with heating to a higher temperature for accelerating the reaction, that is to say, by having really only free organic acids as explained for example in my U. S. Patent 1,217,722 page 4, lines 15 119, 120-129.

Furthermore, I have shown in my said 20 patents that the weaker the condensing agent the more water or similarly acting agents one can use in the secondary reaction for getting given phases of solubilities, not excluding, 25 however, the use of less water or similarly acting agents or no water or similarly acting agents for passing through many more phases of solubilities more slowly and therefore more distinctly, whilst if the condensing 30 agents are stronger the quantities of water or similarly acting agents have to be reduced in order to get certain solubilities based on a given acetylation solution, unless 35 certain or given phase solubilities are to be passed over or never appear.

For the sake of brevity, only these facts are 40 mentioned as having a similar bearing or application here, but for details reference may be had to the above mentioned patents where 45 these matters are fully explained.

By way of example, the further treatment to vary the solubilities of the primary esterification products may be effected by exposing 40 them to the further treatment after first dissolving them in acetic acid or like solvents or after first forming suspensions of them in benzol or like diluents in presence or absence of acetic acid or the like, it being remembered 45 that in conducting the secondary reaction any excess or remaining anhydride has first to be destroyed by water or other anhydride-destroying agents which should preferably be themselves capable of esterification without 50 producing water, e. g. lactic acid, and that the secondary reaction may proceed in the absence or in the presence of water or similarly acting agents, and that according to the quantity of water or similarly acting agents 55 used or present in the secondary reaction, and to the time of reaction and temperature observed, different phases of solubilities can be reached and disappear again according as the reaction is prolonged, it being understood 60 that the less the amount of water or similarly acting agent used the greater will be the range of these phases.

The further treatment or reaction may 65 preferably take place at about ordinary temperature, or as explained in my said patents,

in order to quicken the reaction, one may apply heat or even in some cases heat up to 50° or even 80° to 100° C. (after neutralizing condensing agent that may be present, preferably to the extent of neutral sulphate or neutral salt).

It is to be understood, however, that the various solubilities developed in the secondary reaction or treatment of the products of the present invention do not necessarily correspond to those developed in the products obtained according to my said previous British Patents 20977/1911, 14101/1915, 6463/1915, 100009 and 207562 and U. S. patents Re-issue 14,338, 1,278,885, 1,280,974, 1,280,975 and U. S. application S. 633,016, inasmuch as the primary acetylation products obtainable by the new process of the present invention may have other solubilities than those produced according to my said previous patents.

What I claim and desire to secure by Letters Patent is:—

1. Process for the production of cellulose esters comprising pretreating cellulosic materials with an agent containing vapors of lower fatty acids as sole active agents and thereafter esterifying said pretreated materials substantially in absence of liquid solvents and diluents by subjecting them to the action of vapors of the esterifying agent.

2. Process for the production of cellulose acetates comprising pretreating cellulosic materials with an agent containing vapors of acetic acid as sole active agent and thereafter acetylating said pretreated materials substantially in absence of liquid solvents and diluents by subjecting them to the action of vapors of the acetylating agent.

3. Process for the production of cellulose acetates comprising pretreating cellulosic materials with an agent containing vapors of formic acid as sole active agent and thereafter acetylating said pretreated materials substantially in absence of liquid solvents and diluents by subjecting them to the action of vapors of the acetylating agent.

4. Process for the production of cellulose esters comprising pretreating cellulosic materials with an agent containing vapors of lower fatty acids as sole active agents and thereafter esterifying said pretreated materials substantially in absence of liquid solvents and diluents by subjecting them in presence of a condensing agent to the action of vapors of the esterifying agent.

5. Process for the production of cellulose esters comprising pretreating cellulosic materials with an agent containing vapors of lower fatty acids as sole active agents and thereafter esterifying said pretreated materials substantially in absence of liquid solvents and diluents by subjecting them in presence of a condensing agent to the action of a mixture of vapors of the esterifying agent and an indifferent gas.

6. Process for the production of cellulose esters comprising pretreating cellulosic materials with an agent containing vapors of formic acid as sole active agent and thereafter esterifying said pretreated materials substantially in absence of liquid solvents and diluents by subjecting them in presence of a condensing agent to the action of a mixture of vapors of the esterifying agent and an indifferent gas.

7. Process for the production of cellulose esters comprising pretreating cellulosic materials with an agent containing vapors of acetic acid as sole active agent and thereafter esterifying said pretreated materials substantially in absence of liquid solvents and diluents by subjecting them in presence of a condensing agent to the action of a mixture of vapors of the esterifying agent and an indifferent gas.

8. Process for the production of cellulose esters comprising pretreating cellulosic materials with an agent containing vapors of acetic acid as sole active agent and thereafter esterifying said pretreated materials substantially in absence of liquid solvents and diluents by subjecting them in presence of a condensing agent to the action of a mixture of vapors of acetic anhydride and an indifferent gas.

In testimony whereof I have hereunto subscribed my name.

HENRY DREYFUS.

35

40

45

50

55

60

65